

I. B. LITTLE,  
STORAGE BATTERY GRID MOLD AND MOLDING PROCESS.  
APPLICATION FILED SEPT. 3, 1920.

1,368,445

Patented Feb. 15, 1921.



Fig. 4.

Fig. 5.



16 Inventor,  
Ira B. Little,  
By Joseph A. Minturn  
Attorney.

# UNITED STATES PATENT OFFICE.

IRA B. LITTLE, OF INDIANAPOLIS, INDIANA.

## STORAGE-BATTERY-GRID MOLD AND MOLDING PROCESS.

1,368,445.

Specification of Letters Patent. Patented Feb. 15, 1921.

Application filed September 3, 1920. Serial No. 407,903.

*To all whom it may concern:*

Be it known that I, IRA B. LITTLE, a citizen of the United States, residing at Indianapolis, in the county of Marion and State of Indiana, have invented new and useful Improvements in Storage-Battery-Grid Molds and Molding Processes, of which the following is a specification.

In the casting of double lead grids for storage batteries much loss and waste has been experienced because of the formation of air holes in the frame members of the grid opposite the gate, due largely to the partial filling of that portion of the mold by metal flowing through the middle transverse frame members and reaching the far side of the mold before the air in advance of the metal forming the bottom transverse frame member can fill the latter and rise in the far side of the mold to the level of said middle transverse member. Under the conditions stated it will readily be seen that the air thus cut off from escape will remain to form pockets and air-holes thereby rendering the finished product defective and worthless.

Obviously, the grid-mold must fill from the bottom, up, and all of the comparatively small passages in which the web is formed must be progressively filled in order to avoid air pockets in them. An appreciable length of time is required for the metal to flow from the gate through the small passages of the web and, to keep the fluid metal at a proper temperature so it will not crystallize, and also to provide storage for excess metal coming through the lower passages of the mold while the upper ones are being filled, it has been necessary in common practice to provide a riser of considerably larger capacity than the channel in which the vertical frame member farthest from the gate is formed, and this riser has heretofore been of uniform width and other dimensions from top to bottom, defined by a score line in the same manner as the vertical frame member on the gate side is defined from the gate. But the mold thus formed has resulted in a continuous loss of approximately forty per cent. of output. Many suggestions and experiments in mold-construction have been tried, but without any beneficial results until the application of my invention, which has entirely overcome the difficulty, so that in the manufacture of over a hundred thousand grids with my invention, every one has been

commercially perfect and the former loss has been entirely eliminated.

The object of my invention is to provide a method to cause all of the vertical channels of the mold to fill sufficiently in advance of successive upper horizontal channels to avoid the trapping of air and formation of air holes in the vertical channels.

Another object is gradually to reduce the capacity of the riser from a maximum at a suitable distance above the middle horizontal frame channel to such a suitable minimum at its lower end that the riser will take care of all of the surplus metal and fill to and above said middle channel before the metal coming in from the other end fills said middle channel.

The object also is to reduce the vertical line of communication between the riser and adjacent vertical frame channel to so narrow a dimension that there is not enough room therein for the formation of objectionable air pockets.

I accomplish the above, and other objects which will hereinafter appear, by the mechanism illustrated in the accompanying drawing, in which—

Figure 1, is a view in side elevation of the upper part of a molding table with the molds and their appurtenances assembled in operative closed position. Fig. 2 is an inside view of one half of a mold embodying my invention. Fig. 3, is a transverse section of the complete mold on the line 3—3 of Fig. 2. Fig. 4 is a side view of a casting as it comes from the mold, and before it is trimmed. Fig. 5 shows one of the finished grids, and Fig. 6, is a section on the line 6—6, of Fig. 4.

Like characters of reference indicate like parts in the several views of the drawing.

In the drawing, Fig. 1, 7 is a table to which a standard 8 is bolted, and to which standard the fixed half 9 of the mold is attached. The movable half 10 of the mold is secured to a member 11, hinged at 13 to a depending portion 12 of the standard. The two parts of the mold are forced together by a screw adjustment shown in dotted lines 14, and the mold is opened by grasping handle 14' and swinging on hinge 13 after the pressure is released.

As the channels for the forming of the grid are the same in both mold-halves 9 and 10, except in correspondingly reversed or

110

der, a description of one will suffice for both, it being understood that only half of a grid-forming channel is in each half of the mold.

It will be noted in Fig. 2, that two grids of the form of the finished casting shown in Fig. 5, are cast at one time; also that their abutting frame members in the mold on the line 3—3, make a channel of double size which heretofore has filled its entire length 10 and part way down the frame channel 15, before the metal coming through the frame channel 16 and horizontal web channels 17, have been able to fill channel 15 and connected riser 18. The riser 18 is required, 15 not only to provide storage for excess metal, but more in order to keep the frame formed in channel 15, from cooling to a degree that causes crystallization and weakening of the frame. I separate the riser from the adjacent frame by a channel 19 less than half the thickness of the riser, as shown in Fig. 3, which makes a finished web as shown in Fig. 6, through which the riser is cut from the grids close to the latter, and so narrow 20 that there is not room enough for the formation of objectionable air holes to mar the adjacent frame of the grid.

The dotted lines at the lower portion of riser 18 in Fig. 2, show the extent of the 30 riser channel as same has been heretofore made, and my invention in part, consists in reducing the area of the riser to a minimum of less than half the former width at the bottom, and in gradually tapering the 35 riser to the former maximum width at an appreciable distance above the line of the channel 15.

The shape, size and location of the gate 40 channel 20, is as usual, and in the finished casting the gate-portion is defined from the frame of the grid by a score 21, as a guide in trimming the product.

In the operation of my invention, after 45 the two parts of a mold are closed together, the interference from warping being minimized by recessing the adjacent faces at 22, the molten lead is poured in through the gate channel 20 and begins to fill the mold channels from the bottom. The melted 50 metal flows through the horizontal channels into the vertical frame channel 15, and into the riser 18. From thence to completion, the channels have ample air outlet, and thus the entire casting is made without danger 55 of the confinement of the air that was in them, to form air-holes in the product. The riser channel affords such storage of hot metal in communication with the adjacent vertical frame members through the restricted channel 19, that improper crystallization is prevented, and the web formed in 60 19 is so thin that when cut through in trimming off the surplus metal concealed air

holes thus opened cannot be of any material size.

65

Having thus fully described my invention, what I claim as new and wish to secure by Letters Patent, is—

1. The herein-described method of casting battery grids in vertical molds having vertical channels and horizontal channels connecting the vertical ones, consisting in supplying the melted metal to the bottom of the mold, and filling the vertical channels of the mold sufficiently in advance of successive upper horizontal channels to avoid trapping air and the formation of air holes in the channels.

2. The herein-described method of casting double battery grids in vertical molds having vertical channels and horizontal channels one of the latter of which at the junction of the two grid-molds is of double capacity to form frame-members for two grids, consisting in supplying the melted metal to the bottom of the mold, and filling all of the vertical channels of the mold to the level of said channel of double capacity before the latter channel fills, whereby the trapping of air and formation of air-holes in the casting is avoided.

3. In a mold for casting battery grids said mold having vertical channels and horizontal channels connecting the vertical ones, gate means extending to the bottom of the mold, and a riser of gradually downward reduced area adjacent the far vertical frame member from the gate.

4. The herein described mold for casting battery grids having vertical channels and horizontal channels connecting the vertical ones, gate means extending to the bottom of the mold, a riser of gradually reduced area adjacent the far vertical frame member from the gate connected with said frame by a channel the dimension of which transversely of the mold is less than half that of the adjacent frame member.

5. In a double grid-mold having a double frame channel at the junction of the two grids, a riser having a downwardly tapering lower end which taper begins approximately opposite said double frame channel.

6. In a double grid-mold having a double frame channel at the junction of the two grids, a riser having a downwardly tapering lower end which taper begins approximately opposite said double frame channel and a channel connecting the riser with the mold the dimension of the channel being less than half of the corresponding dimension of the riser.

Signed at Indianapolis, Indiana, this the 28th day of August, 1920.

IRA B. LITTLE.